

## UNITED STATES PATENT OFFICE

FRITZ DOERINCKEL, OF LEVERKUSEN-ON-THE-RHINE, AND LUDWIG MEHLER, OF DORMAGEN-ON-THE-RHINE, GERMANY, ASSIGNEES, BY MESNE ASSIGNMENTS, TO TITANIUM PIGMENT CO., INC., OF NEW YORK, N. Y., A CORPORATION OF MAINE

## PROCESS FOR THE MANUFACTURE OF TITANIUM DIOXIDE

No Drawing. Application filed January 25, 1927, Serial No. 163,556, and in Germany February 1, 1926.

The present invention relates to the hydrolysis of titanium solutions for the manufacture of titanium dioxide which remains white on incandescence.

5 In the manufacture of white titanium dioxide, it is known to separate the same from iron by hydrolytic precipitation from a solution in which all the iron is present in the bivalent condition. When this separation is 10 effected without taking particular precautions, titanic acid or a basic salt of titanium is nevertheless precipitated in a white form, yet at incandescence it assumes a yellow to brown color caused by the small content of iron 15 still contained in the same.

In spite of this disadvantage, a titanium dioxide which remains permanently white at incandescence can be successfully obtained by effecting the reduction to such an extent 20 that not only is all the iron reduced to the bivalent condition, but also part of the titanium to the trivalent form, such for example as has been proposed in German Patents Nos. 152257 and 310304. However these 25 processes involve the disadvantage that only the quadrivalent titanium is precipitated hydrolytically but not the trivalent, which latter therefore is either lost or is only recovered by tedious and expensive processes. It 30 is pointed out in the above mentioned patents that the reduction must of necessity be carried to the point, where a portion of the titanium oxide also becomes attacked, and it is expressly emphasized that reducing 35 agents such as sulfurous acid do not exert a sufficiently far reaching action in this connection.

According to the present invention reducing agents as sulfurous acid, sodium sulfite, 40 sodium thiosulfate, or other reducing agents containing sulfur are employed, that is to say reducing agents for the manufacture of titanium dioxide, remaining white at incandescence, which do not convert quadrivalent titanium into the trivalent form. These 45 reducing agents are applied at least in such concentration that the quantity present not only corresponds to that required for reducing the trivalent iron, but that it must suffice to render innocuous the whole of the

oxidizing agents present in the solution, inclusive of dissolved oxygen from the air. Furthermore care must be taken during the washing process following the hydrolysis that sufficient of said reducing agent must be 55 present in order to prevent a re-oxidation of the iron. By the application of the method of working outlined above, it is now possible to obtain a titanium dioxide, which remains absolutely white at incandescence, by the use 60 of sulfurous acid.

The process can also be effected by first causing reduction to take place with a strong reducing agent which likewise attacks quadrivalent titanium and allowing the reduction to 65 proceed to such an extent, that the whole of the titanium still remains in the quadrivalent form, after which as above described a slight excess of a weaker reducing agent is added and maintained throughout the washing process. So long as the quantity proportions are 70 known the addition of the reducing agents can be effected with equally good results either simultaneously or in any desired sequence.

We claim:

1. In the manufacture of titanium dioxide which remains white at incandescence the step which comprises hydrolyzing a titanium solution in the presence of a reducing sulfur-oxygen compound in a quantity corresponding at least to the trivalent iron and other oxidizing agents present in the solution.

2. In the manufacture of titanium dioxide which remains white at incandescence the step which comprises hydrolyzing a titanium sulfate solution in the presence of sodium sulfite in a quantity corresponding at least to the trivalent iron and other oxidizing agents present in the solution.

In testimony whereof we have hereunto set our hands.

FRITZ DOERINCKEL.  
LUDWIG MEHLER.

95

100